

## UNITED STATES PATENT OFFICE

2,186,509

## FINISHING LEATHER

Fredrick J. Wallace, Erie, Pa., assignor to Robeson Process Company, New York, N. Y., a corporation of New Jersey.

No Drawing. Application July 12, 1938,  
Serial No. 218,881

11 Claims. (Cl. 149—4)

This invention or discovery relates to finishing leather; and it comprises a method of finishing partially tanned leather wherein there is incorporated in the leather a substantial amount 5 of lignin recovered from liquors produced by the digestion of wood with alkaline liquids; and it comprises as a new material finished leather containing substantial amounts of recovered lignin; all as more fully hereinafter set forth and 10 as claimed.

Lignin is a group name for the non-cellulose components of woody fiber. In the acid processes of making paper pulp it reappears in the form of soluble sulfonic acid salts and acids; as ligno- 15 sulfonates which contain sulfur, as the sulfonic group, as an essential constituent. In the alkaline processes of making pulp, the caustic soda process and the sulfate process, it reappears in solution in the "black liquor" withdrawn from the cellulose. This liquor contains lignin as such 20 although the lignin is probably not in a state in which it exists in the wood where it is in combination with cellulose as lignocellulose. This solution is quite impure and ordinarily contains 25 considerable caustic alkalinity; that is, caustic soda over and above the amount in combination with the organics. It also contains all the water-soluble matter of the wood. From the black liquor a tolerably pure form of lignin can be obtained 30 by addition of an acid. The lignin comes out of the solution as a tolerably pure precipitate. Such a precipitate, after washing, is used in the present invention.

It can be redissolved in water containing caustic soda to give a solution containing but little 35 free caustic alkali. Such a solution is advantageous for use in the present invention.

In producing leather, the hides and skins are 40 customarily treated with an infusion of tanning materials or tanning liquors and various procedures are used to obtain the desired degree of tannage. For instance, vegetable tanned sole leather is generally produced by a series of treatments with tanning liquors of various strengths; 45 the strength of the tanning liquors contacted with the hide being gradually increased to a maximum and then gradually decreased in successive steps.

In an ordinary procedure the first stage of 50 tanning is produced by rocking the hides in tanning liquors, the strength of which is gradually increased. The partially tanned hides coming from the rocker yard are then laid away in pits containing tanning liquors of higher concentration, these pits being known as "layers" and the

hide being treated successively in several layers to effect this next stage in the tanning procedure. After removal from the last layer, generally the hides are drummed in a concentrated 5 solution of a tanning agent to complete the tanning. These drums are known as extract wheels, and this treatment with concentrated tanning liquors, that is, strong liquors, is known as drumming or extracting. Tanning liquors are generally known as extracts and this procedure puts 10 extract into the hide. After removal from the extract wheel, the tanned hides are tempered by immersing them in vats containing weaker tanning liquids or solutions. After removal from the last tempering vat, the hides may be wrung, 15 bleached, oiled and dry-dipped prior to finishing. In all stages of the vegetable tanning process, the tanning solutions are of acid character and the tanned hide has a substantially acid reaction, the pH being from 5.0 to 2.5. 20

I have discovered that an increased degree of tannage and other betterments are obtained by incorporating in the tanned hides a substantial amount of lignin as by applying a slightly alkaline lignin solution thereto. This may be done at 25 any stage after the hide has been partially tanned, for instance, after the rocking of the hide in tanning liquors. The slightly alkaline solution of lignin penetrates and impregnates the hide and the natural acids present in the hide 30 gradually neutralize the slight alkalinity of this solution, thus precipitating the lignin in the hide in insoluble form. This addition can be made at any of the stages usually employed in tanning. That is, this incorporation of the lignin may be 35 effected as part of the tanning procedure and I obtain improved leathers irrespective of the particular stage at which the lignin is incorporated. The so treated hides, after the usual operations 40 are completed, yield leathers showing an increased degree of tannage and other improved qualities. 45

However, advantageously the lignin may be incorporated during the extracting or drumming operation, that is, the tanned hides from the last layer may be drummed with alkaline lignin solutions having a pH of approximately 8.2 to 9.2. Such a solution readily penetrates and homogeneously impregnates the moist partially tanned hide during the drumming. Drumming in the 50 extract wheel is continued until the weakly ionized or dissociated natural acids present in the wet hide completely precipitate all of the lignin in insoluble form. Likewise, the lignin may be incorporated in the hide as part of the other op- 55

erations; for instance, during the oiling, that is, introduced as part of the oil wheel load or during the dry dipping, prior to finishing in the usual manner. In dry dipping, the rough dried tanned hide may be dipped in a suitable alkaline lignin solution, and then after the lignin has been precipitated in the hide, it is removed from the solution. Then it may be further processed similarly to the ordinary dry dipped hides to obtain a finished leather. Such incorporation of the lignin after the hides have been tempered is advantageous. The tanning with the usual tanning agent having been completed, the treatment with the slightly alkaline lignin solution can be controlled to produce leathers meeting particular specifications as to degree of tannage and other qualities. In this way leathers having the desired qualities may be reproduced irrespective of variations in the hides and tanning agents employed.

In some cases the precipitated washed lignin may be employed in tanning operations direct, but as a rule I find it better to dissolve it in alkali.

In preparing lignin from black liquor the following procedure is advantageous: The black liquor is treated with sufficient acid to neutralize the alkalinity and to precipitate the lignin. Any acid may be used. After separating the acid mother liquor, the precipitate is washed with water until free of soluble material. The wet precipitate is then dried or dehydrated to remove excess moisture. It may be ground to a powder if desired. So prepared, this lignin is sufficiently free of deleterious materials to be useful in tanning.

For precipitating the lignin I usually employ sulfuric acid, but other suitable mineral or inorganic acids may be employed. The acid treatment of the black liquor in addition to precipitating the lignin also forms volatile sulfides and mercaptan compounds, when some types of black liquors are employed. Volatile and soluble materials are removed during the washing and drying. The following examples are typical illustrations of my methods of recovering lignin useful for my purposes from two types of commercial black liquors.

*Example 1.*—This example illustrates the recovery of lignin from a spent black liquor obtained as a byproduct in treating wood by the kraft process; the liquor having a solid content of 19.10 per cent and a free alkalinity of 2.10 per cent calculated as NaOH.

To 10,000 pounds of liquor were added, with stirring, a solution of 380 pounds of sulfuric acid in an equal amount of water. This acid treatment in this case develops volatile sulfides and mercaptan compounds and precipitates lignin as a brown flocculent material. After the mixture has been thoroughly stirred, it is allowed to settle for two hours. Then the mixture is heated to 160° F. to flocculate and coagulate any lignin remaining suspended in the mother liquor. This heating also drives off some of the volatile sulfides and mercaptans. The mother liquor is then decanted from the lignin which has settled out. The separated lignin is washed with water, dried and ground to a powder. The washing and drying remove water-soluble bodies and volatile materials. In this way approximately 870 pounds of purified lignin are obtained.

Similar lignin preparations useful for the present purposes may be also obtained from the black

liquors resulting from the soda process. This is illustrated in the following example:

*Example 2.*—In this example, a soda process black liquor having a free alkalinity of 2.90 per cent and total solids of 22.29 per cent is employed.

To 10,000 pounds of such black liquor there is added 500 pounds of sulfuric acid dissolved in 500 pounds of water. The lignin is precipitated as a reddish-brown flocculent material. The mixture is agitated for 2 hours and then heated to 160° F. to flocculate and coagulate the precipitated lignin. The lignin is then filtered from the acid mother liquor, thoroughly washed with water and dried. In this way, approximately 810 pounds of dry material is obtained.

The dry lignin preparation obtained in the above examples may be converted into alkaline lignin solutions suitable for treating leather, by suspending the lignin powder in water and then adding just sufficient caustic soda to this suspension to dissolve the lignin. The resulting solutions have a pH value slightly on the alkaline side. Those having a pH value between 8 and 9.2 are advantageous for the present purposes. These solutions can be used as they are in treating leather, or they can be evaporated to a greater concentration. By evaporating to dryness I obtain dry slightly alkaline lignin preparations which are used in treating wet hides, in some modifications of the present invention.

The following examples illustrate the manufacture of these preparations:

*Example 3.*—This example illustrates the preparation of an alkaline lignin solution suitable for dry dipping.

In 1760 pounds of water there is suspended 870 pounds of the lignin powder obtained in Example 1. This mixture is agitated and 52 pounds of sodium hydroxide are added, and the stirring continued until a uniform solution of lignin is obtained. The resulting solution has a pH value of 8.9 and is quite concentrated. When diluted with additional water to a density of 60° barkometer, a solution advantageous for dry dipping is obtained.

*Example 4.*—This example illustrates my methods in improving leather by dry dipping.

The lignin solution of 60° barkometer obtained by Example 3 is heated to 110° F. and rough dried vegetable tanned leather immersed in this solution. The temperature is maintained until the lignin is precipitated in the leather. Approximately one hour is required.

Then the leather is removed and further processed. It is bleached by immersion in water, then in sodium carbonate solution, and finally in sulfuric acid solution, using the ordinary procedures. Thereafter the so treated leather is oiled and dried.

The following table gives the analysis of the treated and untreated leathers:

|                      | Leather before dry dipping in alkaline lignin | Leather after dry dipping in alkaline lignin |
|----------------------|-----------------------------------------------|----------------------------------------------|
| Insoluble ash.....   | .09                                           | .08                                          |
| Moisture.....        | 11.42                                         | 11.17                                        |
| Grease.....          | 2.83                                          | 2.71                                         |
| Hide substance.....  | 41.26                                         | 37.90                                        |
| Water soluble.....   | 15.02                                         | 11.83                                        |
| Combined tannin..... | 29.38                                         | 36.31                                        |
| Total.....           | 100.00                                        | 100.00                                       |
| Degree tannage.....  | 71.2                                          | 95.8                                         |
| pH.....              | 3.03                                          | 4.09                                         |
| Mineral acidity..... | 1.40                                          | .00                                          |

From the above analysis the increased degree of tannage and other improvements obtained by so incorporating the lignin into the leather are evident.

- 5 *Example 5.*—This example illustrates the preparation of an alkaline lignin solution from the lignin recovered from soda process liquor. In 1620 pounds of water there are suspended 810 pounds of the dry lignin powder obtained in 10 Example 2. This mixture is agitated and 40 pounds of sodium hydroxide are added. The agitation is continued until a uniform solution of the lignin is obtained. The resulting solution has a pH value of 9.0 and contains approximately 33 15 per cent by weight of solubilized lignin.

This solution may be used to treat and impregnate leather as described in Example 4. Also, it may be dried to obtain a slightly alkaline lignin powder which is also useful for addition to tanned 20 leather. This may be done by drying the alkaline lignin solution under vacuum and then grinding the dried material to a powder in a ball mill.

- 25 *Example 6.*—This example illustrates the treatment of tanned leather with my dry alkaline lignin powders; vegetable tanned leather prepared by regular tannery methods for the oiling process after bleaching being employed.

This vegetable tanned leather is charged into the usual oil wheel and then the alkaline lignin powder described in Example 5 is introduced into the drum in a ratio of 12 pounds per 100 pounds of dry leather. After the powder has been added the drum is closed and rotated until the powder is thoroughly driven into the leather, about 20 30 minutes drumming being usually required. Then a solution of oxalic acid is added in an amount sufficient to introduce 0.75 pound of oxalic acid for each 12 pounds of lignin powder, and the drum is rotated for an additional 10 minutes. 40 Then the oil is added in the usual way and the drum rotated until the oil is uniformly distributed. After drumming the leather with the oil, it is then dried in the usual way.

The following table gives the analysis of the 45 treated and untreated leathers:

|                  | Leather before drumming with alkaline lignin | Leather after drumming with alkaline lignin |
|------------------|----------------------------------------------|---------------------------------------------|
| 50 Insoluble ash | .12                                          | .11                                         |
| Moisture         | 11.98                                        | 11.63                                       |
| Grease           | 2.64                                         | 3.98                                        |
| Hide substance   | 41.38                                        | 37.02                                       |
| Water soluble    | 14.67                                        | 12.91                                       |
| Combined tannin  | 29.21                                        | 34.58                                       |
| 55 Total         | 100.00                                       | 100.00                                      |
| Degree tannage   | 70.5                                         | 92.7                                        |
| pH               | 3.06                                         | 4.12                                        |
| Mineral acidity  | 1.07                                         | .00                                         |

- 60 In the above example the solution of oxalic acid is added to ensure complete precipitation of the lignin in the leather. In other of my processes I may also add oxalic acid or other organic acids to facilitate the precipitation of the lignin 65 in the hide. For instance, the precipitation of the lignin within the leather may be hastened by the addition to the leather of acid substances such as niter cake, oxalic acid, tartaric acid or other acid materials. Again, in applying the alkaline lignin solutions to the leather in the extract wheel, that is, during drumming, the extract wheel may be opened after the leather is impregnated with the solution and then an acid 70 solution of sodium bisulfate or oxalic acid added 75

and thereafter the wheel rotated for a further period of time to complete the precipitation of the lignin. The acid so added rapidly penetrates the leather and completely precipitates the alkaline lignin in insoluble form upon the leather fiber. Similarly, in my methods wherein the alkaline lignin solutions are applied to rough dried tanned hides by dry dipping, the so treated 10 hides may be subsequently immersed in an acid substance. Such additions of or subsequent treatments with acids are advantageous in treating tanned leathers which have but slight acidity, or in incorporating relatively large amounts of lignin, or both. Usually the tanned leathers are 15 sufficiently acid to fully and completely precipitate the lignin in ordinary operations.

The following example illustrates my processes of drumming with alkaline lignin solutions followed by an acid treatment:

- 20 *Example 7.*—In this example vegetable tanned sole leather taken from the last layer of the tanning process is employed.

25 After rinsing, this vegetable tanned sole leather is introduced into the drum or extract wheel and the alkaline solution obtained in Example 1 is introduced in sufficient amount to give a ratio of 500 pounds of this liquid (33 per cent solids) per 1000 pounds of dry hide. The drum is closed and then rotated until the solution is 30 absorbed by the hide. The drum is then stopped and opened and a solution containing 30 pounds of sodium bisulfate is added. The drum is then rotated for an additional 20 minutes.

The so treated leather is then removed from the drum and immersed in a tanning solution of 60° barkometer for 6 days. After this tempering it is wrung, bleached, oiled and dried.

The following table gives the analysis of the treated and untreated leathers:

|                  | Leather before extracting or drumming in alkaline lignin | Leather after extracting or drumming in alkaline lignin |
|------------------|----------------------------------------------------------|---------------------------------------------------------|
| 50 Insoluble ash | .11                                                      | .10                                                     |
| Moisture         | 12.71                                                    | 12.56                                                   |
| Grease           | 2.87                                                     | 2.94                                                    |
| Hide substance   | 43.41                                                    | 38.44                                                   |
| Water soluble    | 12.18                                                    | 10.16                                                   |
| Combined tannin  | 28.72                                                    | 35.80                                                   |
| Total            | 100.00                                                   | 100.00                                                  |
| Degree tannage   | 66.2                                                     | 98.1                                                    |
| pH               | 3.19                                                     | 4.17                                                    |
| Mineral acidity  | 1.16                                                     | .00                                                     |

55 The leathers obtained by any of the foregoing procedures show a high degree of tannage, a high percentage of combined tannin and a low percentage of a water soluble, as is evident from the tables given ante. The so treated leathers are also advantageous in that they are relatively impervious to changes in atmospheric or climatic conditions, such as changes in humidity. The precipitated lignin contained in the leather is non-hygroscopic and does not absorb moisture. These lignin-treated leathers also have a higher pH value and substantially no mineral acidity or Procter-Searle value. This is also advantageous.

60 The examples given ante illustrate certain embodiments of the present invention. In practising my invention, other embodiments thereof may be employed in commercial practice and in them the various conditions, such as the percentages, concentrations, time, temperature, etc., may be varied according to the particular type of 70 75

leather desired and the particular type of hides or leather being processed. That is, by my broad invention I can improve in various ways all types of tanned hides and leather, including those tanned wholly or partially with natural tannins, such as chestnut, quebracho, cutch, myrobalans, valonia, sumach, wattle, divi-divi, or other natural extracts; or with synthetic tannins such as aromatic sulphonc acids, or sodium salts, or aromatic sulphonc acids partially or wholly condensed with aldehydes or other similar so-called synthetic tannins; or with mineral tanning substances, such as basic chrome solutions or alum. Lignin additions are also useful with leather tanned with sulfite liquor preparations.

15 In the examples given ante, I have described preparing the alkaline lignin solutions from the dried or dehydrated lignin. This is advantageous, but it is not absolutely necessary to dry the wet precipitated lignin prior to forming such solutions. In some embodiments of the present invention, I wash the precipitated lignin, and after filtering off the wash liquors redissolve the wet precipitated lignin in alkaline solutions.

20 25 What I claim is:

1. In the manufacture of leather, the improvement which comprises impregnating tanned leather with recovered lignin from woody fibers, solubilized by alkali, and insolubilizing the lignin in situ in the leather.

2. The process of claim 1 wherein a slightly alkaline lignin solution is applied to a slightly acid tanned leather.

3. As an improvement in tanning leather, the process which comprises drumming tanned hides with a concentrated alkaline solution of recovered lignin from woody fibers, the alkalinity and concentration of said solution being so adjusted that the normal acidity of the tanned 25 30 35 40 hide precipitates the lignin in insoluble form in situ in the hide.

4. In the manufacture of improved leathers,

the process which comprises drumming tanned hides with a concentrated alkaline solution of recovered lignin from woody fibers, having a pH somewhat in excess of 7.0 until the alkaline lignin is absorbed by the leather, adding an acid solution to the so impregnated leather and continuing the drumming until the lignin is precipitated upon the fiber in insoluble form.

5. In the manufacture of improved leather, the process which comprises dry dipping tanned leather in a hot solution of soluble alkalinized recovered lignin from woody fibers, having a pH value somewhat in excess of 7.0.

6. The process of claim 5 wherein the said tanned leather contains sufficient natural acids to precipitate the lignin on the fiber in insoluble form.

7. The process of claim 5 wherein the dry dipped leather is subsequently immersed in an acid solution to precipitate the absorbed lignin in insoluble form.

8. In the manufacture of improved leathers, the improvement which comprises drumming the leather with a dry powdered alkaline lignin having a pH value in excess of 7.0.

9. In the manufacture of lignin preparations suitable for improving leather, the process which comprises acidifying black liquor with sufficient acid to precipitate the lignin, separating the precipitated lignin from the mother liquor, washing the precipitated lignin and treating the lignin so obtained with sufficient alkali to produce a soluble alkaline lignin.

10. The process of claim 9 wherein a concentrated solution of said soluble alkaline lignin having a pH value in excess of 7 is prepared and this solution applied to leather.

11. As a new material a leather made from vegetable tanned hide and carrying incorporated recovered insoluble lignin from woody fibers, in substantial amount.

FREDRICK J. WALLACE.